

Sept. 13, 1932.

F. J. BULASK

1,877,714

## METHOD OF MELTING GLASS

Filed Nov. 18, 1929

3 Sheets-Sheet 1



Inventor  
Francis J. Bulash.

Owen Owen

Attorney's

Sept. 13, 1932.

F. J. BULASK

1,877,714

METHOD OF MELTING GLASS

Filed Nov. 18, 1929

3 Sheets-Sheet 2



By Owen & Owen

Attorneys

Sept. 13, 1932.

F. J. BULASK

1,877,714

METHOD OF MELTING GLASS

Filed Nov. 18, 1929

3 Sheets-Sheet 3



Francis J. Bulash.

By *Owen & Owen*

Attorneys

## UNITED STATES PATENT OFFICE

FRANCIS J. BULASK, OF TOLEDO, OHIO, ASSIGNOR OF ONE-HALF TO GEORGE W. BATCHELL AND FRANZ G. SCHWALBE, BOTH OF TOLEDO, OHIO

## METHOD OF MELTING GLASS

Application filed November 18, 1929. Serial No. 407,960.

This invention relates to a method of and apparatus for melting glass and has for its object to provide a method and apparatus which will simultaneously mix and melt glass materials. More particularly the object of the invention is to expose material added to the furnace to intense heat promptly, thoroughly and uniformly, so as to quickly fuse or melt it, and to thoroughly mix the material prior to, during and subsequent to the melting operation so as to produce a uniform product.

In the accompanying drawings forming a part of this specification, Figure 1 is a vertical longitudinal section of a furnace embodying one form of the invention, with some of the associated parts added. Figure 2 is a plan view of the apparatus disclosed in Figure 1. Figure 3 is a horizontal section of the melting furnace shown in Figure 1. Figure 4 is a partial vertical section of a slightly modified melting furnace employed with different subsequent treatment of the melted material. Figures 5 and 6 are sections on the lines 5-5 and 6-6 respectively of Figure 4. Figure 7 is an end view of the melting furnace as seen from the right of Figure 4. Figure 8 is a diagrammatic plan view of the melting furnace arranged for a different method of heating. Figure 9 is a plan view of a special arrangement of a plurality of melting furnaces of the type shown in Figure 1.

The receptacle for the material being melted, as shown in Figure 1, comprises a casing 10 within which there is a refractory lining 11. Where the heat in the furnace is very high, one or more insulating layers 12 may be provided between the refractory lining 11 and the casing, such insulation acting both to prevent undue waste of heat and also to maintain the casing sufficiently cool to retain its strength.

The casing is provided with supporting and driving rings 13 which are engaged by driving gears 14 on a drive shaft 15 which is suitably connected by gearing 16 to a motor 17. The rings are also supported upon anti-friction wheels, not shown, so that the entire

casing may be rotated about its longitudinal axis.

At the left end of the melting receptacle, as shown in Figure 1, there is a feeding device 18 adapted to feed the material through an opening 19 in that end of the melting receptacle. The right end of the melting receptacle is provided with an opening 20 which is placed in operative relation to a heat producing furnace 21. In the construction shown this heat producing furnace is provided with an air passage 22 and a gas passage 23, the air and gas uniting in a flame which enters the right end of the melting receptacle and is driven to the left end thereof. Some of the products of combustion pass out around the feeding device into a chimney 24, but preferably only a minor part of the products of combustion is led off in this manner, sufficient to prevent any dead areas at that end of the furnace, the greater part of the products of combustion returning as indicated by arrows 25 along the lower side of the melting receptacle and passing downward as indicated by arrow 26 into a runway 27.

The runway 27 is shown as being provided with tracks 28 upon which carriages 29 may be moved, each carriage supporting a pot 30. Beneath runway 27 there is constructed suitable checkerwork 31 through which the products of combustion may be led from the runway to any suitable chimney, not shown, this checkerwork being utilized in any suitable manner for heating the gas and air entering ducts 22 and 23.

In the construction shown the glass melting receptacle and feeding device are mounted upon a base 32 which in turn is supported by wheels 33 upon a track 34 so that the receptacle and feeding device may be moved as a whole towards or from furnace 21.

Rising from base 32 there is a framework 35 supporting the melting receptacle and its drive shaft. Motor 17 likewise is supported upon base 32. From the left end of base 32, as viewed in Figure 1, there rises a framework 36 upon which there is mounted a runway 37 adapted to support feeding device 18.

18 for movement towards and from the receiving end of the melting receptacle.

Surrounding the discharge end of the melting receptacle there is a flange 38 which is adapted to be moved into close proximity to packing 39 mounted against the stationary ring 40 on furnace 21. Beneath the discharge end of the melting receptacle there is a block 41 adapted to act as a spillway for guiding molten glass from the melting receptacle into pot 30. Under the left end of base 32, as viewed in Figure 1, there may be provided a jack 42 or other similar means which may be used for elevating that end of base 32 so as to bring the melting receptacle into proper close relation with the furnace and to form a rigid foundation for the base while the furnace is in actual operation, and for a further purpose which will be described later.

20 In Figure 4 there is shown a slight modification in which the melting receptacle 11' is provided in proper position to discharge material onto the spillway block 41' from which it flows into a plaining tank 43.

25 For convenience the operation of the apparatus will now be described, it being understood that the operation of the device disclosed in Figures 1 and 4 is the same, except in respects which will be pointed out hereafter.

When the apparatus has been assembled as indicated in Figure 1 with the discharge end of the melting receptacle in proper relation to heating furnace 21 and the feeding device 18 in proper relation to the receiving end of the melting receptacle, heat is applied to the interior of the melting receptacle. The flame passing from the upper portion of furnace 21 enters the melting receptacle as indicated by arrows 44. It will be seen that the receptacle comprises a receiving portion 45 and a discharge portion 46, each of which is in the shape of a hollow frustum of a cone, with their bases together at 47. As the flame proceeds longitudinally of the receptacle, it will be readily seen that it will strike against the interior of the receiving portion 45, as indicated by arrow 48, more directly than against the approximately parallel but slightly diverging wall of portion 46. This more direct impingement of the flame against the wall portion 45 highly heats portion 45 of the receptacle.

55 In first starting the furnace it is well to utilize cullet for filling the pores of line 11 and glazing the interior thereof, as is well known in the use of pots and similar glass melting receptacles. When the receptacle is prepared for receiving the glass batch and is properly heated, batch material 49 is fed into the receiving end of the melting receptacle. This material is melted and mixed in the receptacle in a manner which will be described in detail later. The molten glass is discharged in a stream 50 from the discharge

end of the melting receptacle onto block 41 from which it flows downward into pot 30.

Runway 27 is extended for some distance on each side of furnace 21 as indicated in Figure 2. At one end there is provided a receiving chamber 51 divided from the main portion of the tunnel by a gate 52. A pot 53 is placed in the receiving chamber and is gradually heated up in that chamber. The pot is moved to a position on the other side of the gate, as indicated at 54, where it is brought to a temperature approximating that of molten glass. It is then moved to the position occupied by pot 30 and receives the molten glass without exerting any detrimental chilling effect thereon. After being filled, the pot is moved successively to the positions indicated at 55 until it reaches a gate 56 across the discharge end of the tunnel. The pot is then moved past gate 56 to discharge position 57 from whence it may be removed to utilize the molten glass in any desired manner.

90 In Figure 4 there is indicated a melting receptacle 11' substantially the same as shown in Figure 1, but being employed to deliver glass in a somewhat different condition. In this construction the glass stream 50' flows from slab 41' into a refining or plaining chamber 58. This chamber may itself constitute a dog house or gathering chamber or dog house connected thereto, or the glass may be removed therefrom in any suitable manner.

95 It is preferable to heat the melting receptacle in the manner indicated in Figure 1, wherein the fuel is introduced into the upper end of the discharge end of the melting receptacle and impinges against the wall at the receiving end thereof and thereafter is returned to the lower portion of the discharge end, with the exception of a minor amount of the products of combustion which escape in order to prevent any stagnant areas in the receiving end. However, other methods of heating may be utilized if desired. In Figure 8 there is indicated diagrammatically a system wherein the fuel is admitted in the discharge end 59 of the melting receptacle 11' and is discharged from the receiving end 60, 100 from which it is deflected by a gate 61 alternately through different channels for recovering the waste heat by a regenerating system, which will be readily understood without further description. The fuel, flame and products of combustion in such a construction will travel as indicated by arrows 44' in Figure 4.

105 If preferred, the receptacle might be heated by introducing the fuel or flame into the receiving end of the receptacle. In other words, while the method of heating disclosed in Figure 1 has advantages which will be more fully detailed below, the broad aspect of the invention is not confined to this method

of heating the melting receptacle and the contents thereof.

The arrangement shown in Figure 2 may be utilized as a single unit for producing glass for various purposes, but where this type of melting furnace is used in a large factory, a series of melting furnaces may be arranged in connection with pots, as indicated in Figure 9. In this figure there are indicated a plurality of melting receptacles 62, 63, 64, 65, each with a furnace 66, 67, 68, etc., respectively. Adjacent melting receptacles 62 and 63 are arranged with their discharge ends directed in opposite directions and between each such pair of melting receptacles there are a pair of tunnels for pots, there being a tunnel 69, 70, 71, etc., one for each melting receptacle. The pots in each tunnel may be manipulated as discussed in connection with Figure 2, but it is obvious that only one door to the outside is necessary at each end of each pair of tunnels, as the same door may be utilized for removing a filled pot and introducing an empty pot if desired, there being a suitable transfer truck for conveying the pot carrier from one tunnel to the other. This constitutes a compact arrangement in which pots may be taken filled from and returned empty to the same places.

The melting action will now be described in greater detail. As indicated above, the sloping wall of portion 45 of the melting receptacle becomes highly heated. Preferably material 49 is fed into the receptacle in a comparatively thin, broad stream, so as to be exposed to the heat while falling onto the lower side of the receptacle. Whatever the form of the stream, however, it immediately falls upon the sloping wall of portion 45 and becomes highly heated by that wall.

The more easily fusible portion of the batch melts promptly upon being exposed to the heat within the receptacle, and surrounds the less fusible particles mixed therewith. While the heating effect within the receptacle may be modified by proper control of the flames, there is a tendency for the hottest flames and products of combustion to rise to the upper wall, so that ordinarily that is the most highly heated portion of the receptacle; but as the receptacle turns the upper wall is constantly being turned down under the material in the bottom of the receptacle. In normal use, the entire inner surface of the receptacle becomes coated with adherent molten material of the batch, so that heat is applied throughout the interior of the receptacle directly to the batch.

The coating on the upper wall of portion 45 tends, as indicated at 72, to flow towards the entrance end of the receptacle, some reaching block 73, falling onto the upper side 79 of the feed spout, and flowing in a stream 75 down the inner end 76 of the spout at a point spaced inward from the fresh batch stream 49.

The outward flare of the opening in block 73 aids in keeping the molten material from flowing out of that opening.

The part of the batch not melted upon first entrance into the furnace is rolled and tumbled along the bottom of the receptacle in contact with the heated surface of the melted coating, referred to above, and is mixed with the coating and melted thereby. As normally operated, there is normally a comparatively free zone 77 adjacent the feeding spout, the unmolten portion of the batch moving forward into a zone 78, where it is similar to wet sand. Portions of this material carried up by the ascending wall of the receptacle, drop back in chunks 79, as indicated in Figure 5. As the material is mixed and heated and moved forward, and is melted more and more, it becomes first stiffly plastic and then more and more liquid. In the plastic stage a considerable quantity adheres to the ascending wall and strings down in gobs and sheets as indicated at 80.

The material in the bottom of the receptacle tends to move by gravity from opposite sides towards plane 47. As material is carried up by the ascending wall, the direction in which gravity tends to move it gradually changes until, when the level of the axis of the receptacle is reached, it flows downward in a plane parallel with plane 47. As it continues to ascend, it turns more and more away from plane 47, until along the top of the furnace it flows directly away from that plane. During the descent of the wall, the change in direction continues until when the bottom is reached it is towards plane 47 once more. Thus during a rotation of the receptacle the gravity movement of any portion of glass adhered to the wall outside of plane 47 changes direction through 360°.

Considering a portion of the receptacle where there is considerable depth of material, as shown in Figure 5, it will be apparent that the underside 81 moves with the ascending wall, while the upper side 82 rolls or flows downward, according to its consistency or viscosity. Thus the material continually rolls over itself in a wave 83 along the bottom of the receptacle.

The speed at which the material is moved by the ascending wall varies with the diameter of the receptacle and is greatest along plane 47 and lessens at each side thereof. As a combined result of the changing direction of the adherent coating, due to gravity, and viscosity and progressive action of the material just described and the varying action due to the changing diameter and direction of the wall produced by the double frustumal formation of the interior surface of the drum, a very thorough and constant mixing is effected, varying from rolling kneading, pulling or stirring in accordance with the condition of the material. The sand or batch

is rolled into and mixed with the flux and any segregation of large lumps is prevented. At 84, as indicated in Figure 3, a sort of whirlpool action is set up.

There is a more or less definite line 87 between the whirlpool 84 and the less viscous liquid 85, but there is produced an active mixture along this line also. Due to heating and the mixing operation in both the central part of the drum and the part extending to near the outlet of the drum, gaseous materials produced in the reactions of the ingredients form a foam in the more viscous glass. The foam ceases to rotate vertically and floats on the surface of the liquid material and is discharged over the edge of the drum. The continuous formation of the foam causes movement of the foam by displacement as the foam is produced. The more viscous glass in the form of foam thus moves readily over the edge of the outlet of the drum. The foamy character of the viscous glass immediately disappears as it passes over the lip of the drum by reason of its distension due to its elongated movement and the heat and is discharged as a viscous liquid from the drum. Upon discontinuance of supply of batch materials to the drum the drum will quite entirely empty itself by the conversion of the more viscous material into foam which does not adhere to the interior surface of the drum but locates itself at the lowest point in the rotating drum and moves outward towards the outlet of the drum by displacement as it is formed.

The continuous mixing action, besides quickly distributing the applied heat through the mass, insures uniform composition, and also allows the escape of gases. The interior of the receptacle being lined with molten portions of the batch, the application of heat is directly to the batch material, not to walls of a receptacle. The walls of the usual glass tank are corroded chiefly adjacent the upper surface of the glass. There is no corresponding line in the melting receptacle of this invention.

When glass batch is melted in a pot, heat must penetrate, chiefly by conduction, from the pot walls through the batch to the center thereof. In the usual glass melting tank, batch is dumped onto previously molten glass at one end of the tank. Lumps of the unmolten batch are formed, these lumps being coated with the previously molten glass; but the heat penetrates slowly to the middle of the lump. In each case hours elapse between the melting of one portion of the batch and another portion thereof. This necessitates a long heating period and involves a waste of time and heat, and also results in a product that lacks uniformity because the composition of the portions melted at different rates is different, due to volatilization of flux and various other factors affected by the du-

ration of the melting process. This prolific source of difficulties in the methods generally employed in melting glass is eliminated by the prompt application of heat and simultaneous mixing described above.

The action of the furnace can be varied in many ways. Not only the total heat, but the relative application of heat to different zones may be varied by modification of the pressure and composition of the fuel introduced. The rate of feed and the speed of rotation of the receptacle may also vary to regulate the melting and mixing action. Rotation should be sufficiently rapid to insure maintaining a coating over the interior of the melting receptacle, and not so rapid as to hold the material in place by centrifugal force and prevent the mixing action described above. Variation within these limits varies the mixing action.

By controlling the application of flame, the rate of rotation and the rate of feed, the operation may be suited to any particular purpose, and by inspection or sampling, the condition in each successive zone can be ascertained and any undesired action remedied without waiting for the results in the final product.

Ordinarily the axis of the receptacle is maintained substantially horizontal, but it may be tilted by manipulation of jack 42, or by other suitable means. Drops, gobs or waves of material depending from the upper wall move away from plane 47 more rapidly than a substantially even layer on the under wall flows towards plane 47. As a result, the molten material within the receptacle, and in excess of a coating of a thickness to adhere to the upper wall without marked distortion into gobs, etc., tends to flow to the ends. When feeding of fresh batch is stopped, the material within the receptacle continues to flow out until practically all of the mass is discharged. A more rapid discharge may be secured by raising the entrance end of the receptacle. At any time, the passage of material through the receptacle can be hastened by raising its entrance end, other things remaining equal.

In these various ways the condition in which the glass leaves the receptacle can be governed to suit requirements.

In Fig. 4 the glass is shown as being delivered into a comparatively large defining chamber in which the plaining is completed and which may act as the usual refining chamber in a tank furnace.

While there is indicated on the drawings an arrangement whereby the pots are passed through a plaining zone after being filled, it will be readily understood that for some purposes the glass may be utilized with comparatively little plaining after being received in the pot, especially if the melting receptacle is properly manipulated to deliver the glass

in the desired condition. Furthermore the pots may be removed in any desired manner and delivered to a plaining chamber of any preferred construction if it is not convenient to provide the plaining tunnel for the pots in connection with the melting receptacle.

While the melting of the material in a receptacle such as described may be varied quite materially according to the nature of the glass being melted and the conditions which it is desired to obtain, it will appear from what has been said above that the melting action is accomplished quite promptly. For example, it has been found that in a furnace of the type described, a glass batch suitable for forming plate glass may be melted and reduced within one hour to a condition which would correspond to about seven to nine hours in a melting pot.

For optical glass and other materials where direct contact of the flames and products of combustion is undesirable, means may be employed for heating the outside of the receptacle. Such application of heat is more detrimental to the receptacle and less efficient than the preferred method, but is more efficient than the usual form of muffle pot, and the advantages of the mixing action are retained. While the continuous operation described above is preferred, the apparatus may be operated by the intermittent method where desired, and in any case the discharge may be effected in a continuous stream, in gobs, or in any other manner suitable to the circumstance.

In the operation of the rotary double frustumal receptacle in which the glass mass is heated, the batch materials are first mixed with the fritted glass and the mixture mixes with the semi-molten glass and the molten glass, as it increases in fluidity and viscosity, adheres to the surface of the receptacle, it being drawn from the lower stratum of the glass mass and delivered from the delivery frustum, progressively. When feeding of batch materials cease, continued heating and rotation of the receptacle will cause practically all of the mass to be completely discharged.

What is claimed is:

1. The method of melting glass which consists in progressively feeding batch materials to a heated mass of glass, rotating the mixture in a vertical plane and also in a horizontal plane and progressively separating and removing the molten glass from the mixture.

2. The method of progressively melting glass which consists in progressively feeding batch materials into previously heated fritted glass mass and rotating the glass and batch material mixture both vertically and horizontally, and progressively separating and removing the molten glass from the mixture.

3. The method of heating glass which consists in progressively feeding batch material

into a previously heated glass mass continuously rotating the glass mass and batch material mixture in a vertical plane and also in a horizontal plane and progressively separating and removing the glass mass from the horizontally rotating mass as the viscosity of the glass increases.

4. A method of heating glass which consists in feeding glass batch material into a heated semi-fused glass mass, continuously rolling the batch materials into the semi-fused glass mass to mix the batch materials with the semi-fused mass and carrying portions of the fused mass of increased viscosity upwards and allowing it to fall into lower portions of the fused mass of slightly less viscosity and carrying portions of glass of still higher viscosity over and allowing it to fall into the body portions of glass of substantially the same viscosity and separating and removing and discontinuing rotation of molten glass of predetermined and highest viscosity from the glass of lower viscosity and returning molten glass of lower viscosity towards the rotating semi-fused glass mass and away from the delivery point.

5. The method of progressively melting glass which consists in progressively feeding batch materials into previously heated fritted glass mass and rotating the glass and batch material mixture both horizontally and vertically, and progressively forming a foam from the molten glass and continuously removing the molten foamy glass from the mixture.

6. The method of heating glass which consists in progressively feeding batch material into a previously heated glass mass, continuously rotating the glass mass and batch material mixture in a vertical plane and also in a horizontal plane and forming a foam and continuously removing the glass of the foam from the glass mass by the displacement of the previously formed foam as the foam is created.

7. The method of heating glass which consists in progressively feeding batch material into a previously heated glass mass, continuously rotating the glass mass and batch material mixture in both vertical and horizontal planes and progressively forming a foam from the glass as its viscosity increases and continuously removing the more viscous glass.

8. The method of heating glass which consists in progressively feeding batch materials into a previously heated glass mass, continuously rotating the glass mass and glass material mixture in a vertical plane and also in a horizontal plane and progressively forming a foam that ceases to vertically rotate and continuously discharging the previously formed foam by the foam as it is created.

9. The method of melting glass which consists in progressively feeding glass batch ma-

aterials into a heated fused glass mass, producing rotation of the glass mass and batch material mixture in a vertical plane, progressively separating and removing portions of the glass mass as it reaches a predetermined viscosity from the rotation, and moving progressively the molten glass material towards the delivery point of the glass as the viscosity of the glass increases and continuously preventing movement of the molten glass to the delivery point until its viscosity increases and forming a foam that floats on the less viscous glass.

10. The method of melting glass which consists in progressively feeding glass batch materials into a heated glass mass and producing rotation of the glass mass and batch material mixture in vertical planes and progressively moving the portions of the glass batch material away from the central zone of the glass mass and batch material mixture towards a glass discharging point where the glass is removed from the melting glass as the viscosity of the glass increases and moving the glass mass of lower viscosity away from the said discharging point and forming a foam on the surface of the lower viscous glass and continuously discharging the glass of the foam from the glass discharging point.

11. The method of progressively melting glass which consists in continuously feeding glass materials into a previously heated glass mass continuously heating the glass mass and batch materials and thereby continually changing the adherability and viscosity of the glass mass, continuously rotating the glass mass batch material both vertically and horizontally and progressively separating and removing the glass mass from the mixture and from rotation as its viscosity reaches a certain point while maintaining the rotation of the glass mass.

12. The method of progressively melting glass which consists in progressively feeding glass materials into previously heated glass mass continuously heating the glass mass and batch material and thereby varying the adherability and viscosity of the glass mass, continuously rotating the glass and batch materials both vertically and horizontally forming a foam from the more viscous glass and discharging the glass of the foam as the foam is formed.

13. A method of heating glass which consists in feeding glass batch materials into a heated fused glass mass, continuously heating and rolling the batch materials into the fused glass mass to mix the batch materials of the fused mass and thereby varying the adherability and viscosity of the glass, carrying portions of the more adherable glass forward and allowing it to fall into lower portions of the glass mass, and forming foam

from the more viscous glass and progressively removing portions of the glass foam.

In testimony whereof I have hereunto signed my name to this specification.

FRANCIS J. BULASK. 70